

Aug. 15, 1933.

A. A. GOBEILLE  
ELASTIC WOVEN FABRIC  
Filed July 28, 1932

1,922,944

*Fig. 1.*



*Fig. 2.*



*Fig. 3.*



INVENTOR.

Alfred A. Gobeille  
BY Barlow & Barlow  
ATTORNEYS.

## UNITED STATES PATENT OFFICE

1,922,944

## ELASTIC WOVEN FABRIC

Alfred A. Gobeille, Shannock, R. I., assignor to  
Columbia Narrow Fabric Company, Shannock,  
R. I., a Voluntary Association of Rhode Island

Application July 28, 1932. Serial No. 625,347

19 Claims. (Cl. 139—421)

This invention relates to an elastic woven fabric and is similar in many respects to and is a continuation in part of my co-pending application 603,723, filed April 7, 1932.

5 One of the objects of this invention is to provide a generally flat relatively wide elastic fabric when taken from the loom which may be made unusually thin and formed either relatively flat or shirred thereafter.

10 Another object of this invention is the method of forming a fabric of threads which are shrunk after being woven, by which arrangement I may obtain a more elastic and thinner material than where the threads are shrunk prior to weaving.

15 A further object of the invention is the provision of a fabric with elastic threads such that when the inelastic threads are shrunk the elastic threads will contract and be extendible to the size of the fabric prior to shrinking.

20 A still further object of the invention is to provide a fabric having rubber threads which may contract slightly when taken from the loom but which will have its major contraction in the finishing process.

25 This invention further consists in the method of forming an elastic fabric which, after being taken from the loom, is in an inelastic state and is rendered elastic by treatment in the finishing process.

30 With these and other objects in view the invention consists of certain novel features in the construction and method of forming the fabric as will be more fully described and particularly pointed out in the appended claims.

35 In the accompanying drawing:—

Fig. 1 is a top plan view of a fragmental portion of the fabric showing at its upper portion the fabric as it comes from the loom, and at its lower portion the fabric after it has been finished and shrunk.

40 Fig. 2 is a diagrammatic view of the strands of fabric showing their interweaving relation.

Fig. 3 is a detail view of one of the elastic strands showing the covering thereabout.

45 Fig. 4 is a diagrammatic view illustrating the interweaving relation of the elastic and non-elastic strands in stretched relation.

Fig. 5 is a view similar to Fig. 4 showing the strands in contracted relation.

50 In the use of elastic fabric, it is desirable, especially for summer use in women's garments, such as corsets or the like, to provide thin material, and it has been usual in the formation of such material to use elastic and non-elastic threads which will contract upon being taken from the loom

in which they are woven under tension, and I have found that by weaving the unshrunk threads, which extend at right angles to and also in the same direction as the elastic threads, and using some sizing in these threads that the fabric 60 will not contract any appreciable extent upon being taken from the loom until they are treated in a manner to shrink the threads and remove the sizing from them, whereupon the elastic threads are permitted to contract and a very thin fabric 65 is produced which is desired for the purposes above stated the same being either flat or otherwise depending on the arrangement of the elastic threads; and the following is a detailed description of the present embodiment of this invention 70 illustrating the preferred means by which these advantageous results may be accomplished.

With reference to the drawing, for the sake of convenience, I will designate one component set of threads 10 as warp threads and the other 75 component set of threads 11 as weft threads, although these threads may be interchanged for convenience or the obtaining of different weaves.

In the weft threads there is provided a pair 80 of yarn or relatively non-elastic threads 12 alternating with a pair of relatively elastic threads 13, each of which may be formed with a rubber or latex core 14 and a covering 15 of a textile material usually of the same material as the non-elastic thread 12. In this manner of positioning the elastic and non-elastic weft threads, the elastic threads are sufficiently close together so that when contraction occurs the fabric will remain substantially flat or in a single plane. 85

One convenient form of weaving is to cause 90 weft threads to extend alternately under and over groups 16 and 17 of warp threads which I have here illustrated as three threads included in each group, and when in woven condition, as illustrated 95 in Fig. 4, the elastic and non-elastic threads will be related as there shown when taken from the loom. The non-elastic threads 12 as well as warp threads 10 contain a sizing or gum which causes the fabric to be relatively stiff so that when the 100 fabric is removed from the loom with the elastic strands 13 in stretched condition this fabric will not appreciably change but will remain stiff with the rubbers or elastic threads in the stretched condition which they assume in passing through 105 the loom. This invention has to do primarily with silk or rayon threads, although other materials may be used and the gum or sizing is that usually present in the working of this material. It will also be understood that the elastic threads 110

may be present in the warps as well as in the filling, if desired.

In finishing, the gum or sizing is washed from the non-elastic threads and this washing operation shrinks the non-elastic threads so that the rubber or elastic thread contracts and takes up this shrinkage and the fabric is narrowed by a material extent. It is found that a piece of silk fabric which is woven on a loom substantially 10 forty three inches wide will contract to a width of substantially twenty four inches after being finished and shrunk, although it will be realized this dimension is merely illustrative and not any way confining as to the invention herein disclosed.

15 The elastic threads may be of rubber or latex and the non-elastic threads may be twisted to different degrees with their corresponding binding effect as disclosed in the copending application here and above referred to, where a high twist of the relatively non-elastic threads is disclosed. The fabric thus formed may be used in undergarments and will stretch and snugly fit the body which is desired in many uses of the 20 same.

25 The foregoing description is directed solely towards the construction and method illustrated, but I desire it to be understood that I reserve the privilege of resorting to all the changes to which 30 the fabric is susceptible, the invention being defined and limited only by the terms of the appended claims.

I claim:—

35 1. A method of forming an elastically extendible material, which consists in weaving textile threads having gum or sizing therein with relatively elastic threads of rubber under tension said textile threads being sufficiently close together and containing sufficient gum or sizing 40 to provide a substantially non-elastic fabric when taken from the loom, and then degumming the fabric to permit it to contract and be elastically extendible.

45 2. A method of forming an elastically extendible material, which consists in weaving in the warp textile threads having gum or sizing therein with relatively elastic rubber threads under tension in the weft said textile threads being sufficiently close together and containing sufficient 50 gum or sizing to provide a non-elastic fabric when taken from the loom, and then removing said gum or sizing from the fabric to permit it to contract and be elastically extendible.

55 3. A method of forming an elastically extendible material which consists in weaving raw silk threads with relatively elastic threads of rubber under tension said silk threads being sufficiently close together to provide a substantially non-elastic fabric when taken from the loom, and then degumming the fabric to remove the gum in the raw silk to permit it to contract and be elastically extendible.

60 4. The method of forming an elastically extendible material, which consists in weaving raw silk threads with rubber threads under tension said silk threads being sufficiently close together to maintain the rubber threads under substantial tension and subsequently removing the gum of the raw silk to finish the fabric so formed.

65 5. The method of forming a flat elastic fabric of fine texture, which consists in weaving textile threads having a gum or sizing therein with relatively elastic threads of rubber under tension and spaced in the fabric so as to have an even drawing effect and cause the fabric to be substantially

flat thus providing a non-elastic fabric when taken from the loom and then removing said gum or sizing to permit it to contract and be elastically extendible and yet be substantially flat.

6. An unfinished non-elastic woven fabric 80 formed of rubber threads under tension and raw silk threads said silk threads being sufficiently close together to maintain the rubber threads under tension.

7. An unfinished non-elastic woven fabric 85 formed of rubber threads under tension and highly twisted raw silk threads said silk threads being sufficiently close together to maintain the rubber threads under tension.

8. An unfinished non-elastic woven fabric 90 formed of rubber threads under tension and raw silk threads, said silk threads being sufficiently close together to maintain the rubber threads under tension said fabric being capable of contracting its area upon being moistened.

9. An unfinished non-elastic woven fabric 95 formed of rubber threads under tension and raw silk threads, said silk threads being sufficiently close together to maintain the rubber threads under tension said fabric being capable of contracting its area upon removal of the gum in the raw silk.

10. An unfinished non-elastic woven fabric 100 formed of rubber threads under tension and highly twisted raw silk threads, said silk threads 105 being sufficiently close together to maintain the rubber threads under tension said fabric being capable of contracting its area upon being moistened.

11. A woven fabric formed of component 110 threads extending generally in right angular directions some of the threads extending in one direction being elastic rubber threads and under tension and some of the other component threads being highly twisted and having a removable sizing 115 therein and sufficiently close together to maintain the rubber threads under tension.

12. A method of forming an elastically extendible material, which consists in weaving rubber threads under tension with relatively non-elastic textile threads located sufficiently close together and having a sufficient gum or sizing 120 therein to hold the elastic threads under substantial tension when woven and taken from the loom, and then degumming the fabric to permit a 125 contraction of the rubber threads and provide an elastically extendible fabric.

13. A method of forming an elastically extendible material which consists in weaving rubber threads under tension with relatively non-elastic textile threads located sufficiently close together and having a sufficient gum or sizing 130 therein to hold the elastic threads under substantial tension when woven and taken from the loom, and then degumming the fabric to permit a contraction 135 of the rubber threads and an elastically extendible fabric, said spacing of the non-elastic threads and amount of gum present being such that a major portion of the contraction in the 140 fabric occurs after the degumming step.

14. An unfinished fabric of woven material comprising relatively non-elastic threads having a gum or sizing therein and relatively elastic threads of rubber stretched under tension with 145 the elastic threads maintained under tension by the spacing of and amount of gum or sizing in the relatively non-elastic threads, said fabric being contractible an amount equal to the major portion of its extendibility in the finished fabric 150

upon the removal of said gum or sizing in finishing the fabric.

15. A fabric formed of woven material comprising relatively non-elastic threads and relatively elastic threads of rubber stretched under tension said non-elastic threads being sufficiently close together and containing sufficient gum or sizing therein to maintain the elastic threads under tension.
- 10 16. A fabric formed of woven material comprising relatively non-elastic warp threads and relatively elastic threads of rubber in the weft stretched under tension said non-elastic threads being sufficiently close together and containing sufficient gum or sizing therein to maintain the elastic threads under tension and contractible upon the removal of said gum or sizing.

17. A fabric formed of woven material comprising relatively highly twisted non-elastic warp threads and relatively elastic threads of rubber in the weft stretched under tension said non-elastic threads being sufficiently close together and containing sufficient gum or sizing

therein to maintain the elastic threads under tension.

18. A fabric formed of woven material comprising relatively highly twisted non-elastic threads and relatively elastic threads of rubber stretched under tension said non-elastic threads being sufficiently close together and containing sufficient gum or sizing therein to maintain the elastic threads under tension, and contractible upon the removal of said gum or sizing.

19. A fabric formed of woven material comprising relatively non-elastic threads and relatively elastic threads of rubber stretched under tension, said elastic threads being spaced in the fabric so as to have an even drawing effect and said non-elastic threads being sufficiently close together and containing sufficient gum or sizing therein to maintain the elastic threads under tension said elastic threads being contractible upon removal of said gum or sizing to produce a substantially flat fabric by reason of the even drawing effect of said elastic threads.

ALFRED A. GOBEILLE.

|    |     |
|----|-----|
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |